

# UNITED STATES PATENT OFFICE.

JOHANNES M. KESSLER, OF WEST ORANGE, NEW JERSEY, ASSIGNOR TO E. I. DU PONT DE NEMOURS & COMPANY, OF WILMINGTON, DELAWARE, A CORPORATION OF DELAWARE.

## NITROCELLULOSE COMPOSITION.

1,357,876.

Specification of Letters Patent. Patented Nov. 2, 1920.

No Drawing.

Application filed December 6, 1919. Serial No. 343,047.

To all whom it may concern:

Be it known that I, JOHANNES M. KESSLER, a citizen of the United States, and a resident of West Orange, in the county of Essex and 5 State of New Jersey, have invented certain new and useful Nitrocellulose Compositions, of which the following is a specification.

This invention relates to nitrocellulose compositions containing as a softening 10 agent for the nitrocellulose an ester of an acyloxy derivative of an aliphatic acid, and particularly of a higher fatty acid.

One object of the invention is to provide a composition which may be made into 15 strong and flexible sheets and films that are practically unaffected by water, and that are able to withstand the action of sunlight and air for long periods without appreciable deterioration. Other objects will be apparent from the following description.

A factor of great importance in the manufacture of pyroxylin plastics is the substance used as the softening or conditioning agent for the cellulose ester. Although the 25 patent literature discloses a very large number of substances as substitutes for camphor, only a small number have found practical application. Only a few of these substances show any superiority over camphor, 30 and in these cases the difference is usually insufficient to make up for their much higher cost. About the only one at present available in this country is triphenylphosphate which is employed to a limited extent in the 35 nitrocellulose plastic industry, and then only in connection with camphor.

The scarcity and high cost of camphor has led me to investigate the suitability of 40 various substances as camphor substitutes which have not heretofore been suggested for this purpose; as a result of this investigation I have discovered that cellulose ester sheets and films having excellent physical and chemical properties from the stand- 45 point of their use in the arts may be obtained by using as a softener any one of several classes of substances which may be produced from available raw materials at a reasonably low cost.

50 One of these classes of substances which I have found to be suitable as camphor substitutes, and to which in combination with nitrocellulose, the present application is directed, comprises the esters of acyloxy de-

rivatives of aliphatic acids, and especially 55 of monobasic aliphatic acids containing more than three carbon atoms. The acyl group is preferably either an aliphatic group with a small number of carbon atoms such as formyl, acetyl, and propionyl, or a 60 carbocyclic acyl such as benzoyl. As esters there may be used the glycerid of the acyloxy fatty acids or the corresponding alkyl or aryl esters. For alkyl radicals I prefer those which are readily obtainable 65 such as methyl, ethyl, butyl, etc.; and for aryl radicals; phenyl and alpha- or beta-naphthyl.

The acyloxy derivatives of the lower aliphatic acid esters are not suitable as camphor substitutes or softeners on account of their relative low boiling point, which, in the case of ethyl acetylglucolate ( $\text{CH}_3\text{CO.OCH}_2\text{CO.OC}_2\text{H}_5$ ) is 179° C., and in the case of ethyl acetylacetate ( $\text{CH}_3\text{CO.OCH}(\text{CH}_3)\text{CO.OC}_2\text{H}_5$ ), is 177° C. at 733 millimeters of mercury pressure.

The esters which I have found to be particularly suitable as softeners are the esters of acyloxy derivatives of the higher fatty 80 acids. Examples of such substances are the alkyl esters of mono-, di-, or triacyloxy-stearic acid, and the alkyl esters of acetyl-oxy-oleic acid (that is alkyl acetylricinoleates). The methyl and ethyl esters are 85 preferred, although the glycerid esters have the advantage that they can be obtained directly from the corresponding glycerids (hydroxystearin, ricinolein, etc.) by acetylation of these oils with acetic anhydride. 90

The properties which the new softeners impart to pyroxylin are very remarkable. Without the use of any camphor the methyl and ethyl acetylricinoleates form with nitrocellulose a pyroxylin plastic having an exceedingly great flexibility and pliability. For example I have found that this plastic material has a Schopper number (resistance to cracking on repeated folding) of 170 as compared with 20 for regular transparent 100 pyralin or celluloid.

My invention may be illustrated by the following example: 100 parts (by weight) of dry nitrocellulose are kneaded with 32 parts of methyl acetylricinoleate and from 105 60 to 70 parts of denatured alcohol at a temperature preferably between 40 and 55° C. until the nitrocellulose is properly col-

loided, after which it is put on rolls and through the different operations such as rolling, cake pressing, sheeting and seasoning which are well known in the manufacture of 5 pyroxylin plastics such as pyralin, celluloid, etc. Suitable amounts of stabilizer, for example urea, and of pigments and colors may be incorporated either during the mixing or the rolling operation.

10 The proportions of the ingredients may be varied considerably without departing from my invention; thus, from 28 to 35 parts of the alkyl acetylricinoleate may be combined with 100 parts of the cellulose ester with 15 good results, although I prefer to have the ratio of nitrocellulose to softener equal about 3 to 1. A part of the alkyl acyloxy aliphatic acid ester may be replaced by camphor or other camphor substitute such as 20 triphenyl phosphate.

For producing very flexible films such as are required in the artificial leather industry, a nitrocellulose solution may be prepared in accordance with my invention having 25 the following composition:

30 Nitrocellulose (preferably dry) 10 parts  
Ethyl acetylricinoleate 10 to 15 parts  
Ethyl acetate 40 parts  
Benzene 60 parts

The proportions of the volatile solvents in the above formula may be made greater or less depending upon the viscosity desired, and part of the ethyl acetate may with 35 advantage be replaced by a higher alkyl acetate such as butyl or amyl acetate.

Coating solutions may be prepared using 40 various solvents other than those mentioned above, for example, methyl or ethyl alcohol and acetone. Sheets or films having excellent properties may readily be prepared by flowing the above mentioned solutions on to smooth surfaces and causing the solvent to evaporate.

45 I claim:

1. A composition consisting essentially of nitrocellulose and a softener comprising an ester of an acyloxy derivative of a monobasic aliphatic acid having more than three 50 carbon atoms.

2. A composition consisting essentially of nitrocellulose and an alkyl ester of an acyloxy derivative of a monobasic aliphatic acid having more than three carbon atoms.

55 3. A composition consisting essentially of

nitrocellulose and a softener comprising an ester of an acyloxy derivative of a monobasic aliphatic acid having more than three carbon atoms.

4. A composition comprising a cellulose 60 ester and an alkyl ester of an acyloxy derivative of a higher fatty acid.

5. A composition comprising nitrocellulose and an alkyl ester of an acyloxy derivative of a higher fatty acid.

6. A composition comprising nitrocellulose and a methyl ester of an acyloxy derivative of a higher fatty acid.

7. A composition comprising nitrocellulose, an ester of an acyloxy derivative of a higher fatty acid, and a solvent therefor.

8. A composition comprising nitrocellulose, an ester of an acyloxy derivative of a higher fatty acid, and a solvent therefor comprising an alkyl acetate and benzene.

9. A composition comprising nitrocellulose, an alkyl acetylricinoleate, and a solvent for said substances comprising an alkyl acetate and benzene.

10. A composition comprising 3 parts of 80 nitrocellulose and at least about 1 part of a softener comprising an alkyl ester of an acyloxy derivative of a higher fatty acid.

11. A composition comprising 3 parts of nitrocellulose and at least about 1 part of 85 ethyl acetylricinoleate.

12. A composition comprising nitrocellulose and an alkyl ester of an acyloxy derivative of a fatty acid having 18 carbon atoms.

13. A composition comprising nitrocellulose and an alkyl ester of an acyloxyoleic acid.

14. A composition comprising nitrocellulose and ethyl acetylricinoleate.

15. A composition consisting essentially 95 of nitrocellulose and a softener comprising camphor and an alkyl ester of an acyloxy derivative of a higher fatty acid.

16. A flexible sheet of material comprising nitrocellulose and an alkyl ester of an 100 acyloxy derivative of a higher fatty acid.

17. A flexible sheet of material comprising nitrocellulose and an alkyl ester of acetylricinoleic acid.

18. A flexible material comprising nitrocellulose and a softener therefor comprising an alkyl acetylricinoleate.

In testimony whereof I affix my signature.

JOHANNES M. KESSLER.